

# United States Patent [19]

Ikegaya et al.

[11] 3,860,503

[45] Jan. 14, 1975

[54] **METHOD FOR FORMING A COLORED COATING ON ALUMINOUS MATERIALS**

[75] Inventors: **Masashi Ikegaya; Fumio Shigeta**, both of Shizuoka, Japan

[73] Assignee: **Riken Light Metal Industries Co., Ltd.**, Magarikane, Shizuoka, Japan

[22] Filed: **July 27, 1972**

[21] Appl. No.: **275,821**

[30] **Foreign Application Priority Data**

July 30, 1971 Japan..... 46-57348  
Aug. 21, 1971 Japan..... 46-63337  
Aug. 21, 1971 Japan..... 46-63338  
Aug. 21, 1971 Japan..... 46-63339

[52] **U.S. Cl.** ..... 204/58

[51] **Int. Cl.** ..... C23b 9/02

[58] **Field of Search** ..... 204/58

[56] **References Cited**

UNITED STATES PATENTS

1,735,286 11/1929 Kujirai et al. ..... 204/58

|           |         |                     |        |
|-----------|---------|---------------------|--------|
| 2,150,395 | 3/1939  | Nagata.....         | 204/58 |
| 3,252,875 | 5/1966  | Economy.....        | 204/58 |
| 3,328,274 | 6/1967  | Bushey et al. ....  | 204/58 |
| 3,405,042 | 10/1968 | Neunzic et al. .... | 204/58 |

**FOREIGN PATENTS OR APPLICATIONS**

|         |         |                    |        |
|---------|---------|--------------------|--------|
| 970,500 | 9/1964  | Great Britain..... | 204/58 |
| 802,878 | 12/1968 | Canada.....        | 204/58 |

**OTHER PUBLICATIONS**

"The Surface Treatment and Finishing of Al and its Alloys" by Wernick et al., 3rd Ed., 1964, p. 363.  
"Surface Treatment of Al & its Alloys," Wernick et al., 3rd Ed., 1964, pp. 306, 758-759.

*Primary Examiner*—R. L. Andrews

*Attorney, Agent, or Firm*—Eric H. Waters

[57]

**ABSTRACT**

Colored oxide coatings from yellow to brown on aluminum or aluminum alloy are formed by an anodic oxidation with an aqueous solution of 0.5 – 10.0 percent by weight of oxalic acid and 0.05 – 4.0 percent by weight of an ammonium salt, a metal acetate or a metal nitrate.

**7 Claims, No Drawings**

## METHOD FOR FORMING A COLORED COATING ON ALUMINOUS MATERIALS

The present invention relates to a method for forming a colored oxide coating on the surfaces of aluminum or aluminum alloy materials and particularly a method for forming a colored oxide coating having a broad yellowish color tone on aluminum or aluminum alloy materials by an anodic oxidation.

In the specification, aluminum or aluminum alloys are referred to as merely "aluminous material(s)."

Recently, aluminous building materials have been utilized broadly, because aluminous materials have excellent abrasion resistance and weather resistance and fulfill the requirements desired of building materials and have a beautiful appearance and a broader coloration range than the other metal materials.

However, it can be said that, while the coloration range of aluminous materials is broader than that of the other metal materials it is not always possible to color such aluminous materials in various color tones to the maximum desired extent. Thus, various investigations have been made to widen the color tone but a satisfactory method which can color the aluminous materials to the color tones desired by the user and particularly to a broad range of yellowish color, has never heretofore been developed. Among the processes known for coloring aluminous materials yellow are the following features:

1. Oxalic acid is used as an electrolytic bath.
2. Anodic oxidation is effected in an electrolytic bath containing an aromatic sulfonic acid and sulfuric acid or a metal sulfate.
3. An aluminous material is previously subjected to an anodic oxidation and then applied with an alternate current in an electrolytic bath containing a metal salt.

In any of the above known processes, the obtained range of the color tones is narrow and for example, in the above described first process which is the most practical process among these known processes, the color tone of the obtained oxide coating is of a very narrow range and even if the thickness of oxide coating or the quality of aluminous materials is varied, the remarkable variation in color cannot be obtained. Accordingly, colored oxide coatings having the broad yellowish color tone required by the user, have not heretofore been obtained.

The above described second and third processes can provide oxide coatings having a relatively broad color tone but the second process uses an electrolytic bath consisting mainly of an aromatic sulfonic acid which is a specific chemical and therefore the electrolytic bath is expensive. In the third process, after the usual anodic

The present invention aims to solve the above described deficiencies and provides a method for producing colored oxide coatings of aluminous materials wherein colored oxide coatings of aluminous materials having a broad yellowish color tone are formed by an anodic oxidation using an electrolytic bath having a simple composition.

For the practice of the method of the present invention, firstly, an aluminous material to be treated is degreased with an aqueous solution of sodium hydroxide and then washed with water and successively neutralized in an aqueous solution of nitric acid and then washed with water. Then, the thus treated aluminous material is subjected to an anodic oxidation with direct current by using an aqueous solution containing 0.5 – 10.0 percent by weight of oxalic acid and 0.05 – 4.0 percent by weight of ammonium salt, 0.05 – 1.5 percent by weight of acetate or 0.05 – 0.7 percent by weight of nitrate as an electrolytic bath.

In this case, the above limitation of the composition of the electrolytic bath is based on the following reason.

The addition of oxalic acid serves to improve the electric conductivity of the bath and facilitate the electrolysis, whereby the yellow oxide coating is formed on aluminous materials. This has been previously known as shown in the above described first process. Accordingly, for the same reasons as in the above first process, oxalic acid is added as an essential component of the bath, i.e., in order to obtain the yellow color tone and at least 0.5 percent of oxalic acid is necessary to generate the yellow color; when the amount of oxalic acid is larger than 10.0 percent, the dissolution of such an amount of oxalic acid is difficult at room temperature.

The addition of ammonium salts, acetates or nitrates serves to widen the color range of the oxide coating on aluminous materials and to obtain an yellowish color tone and these salts improve the luminosity. An amount less than the lower limit cannot develop the effect of addition, while even if amounts more than the upper limits are added, the effect of coloration does not vary. It has been found that these ranges can provide colored oxide coatings of a broad color tone from yellow to greyish yellow.

As an ammonium salts, use can be made of ammonium phosphate and ammonium dichromate.

As acetates, use can be made of manganese acetate and chromium acetate.

As nitrates, use can be made of ferric nitrate and chromium nitrate.

The optimum conditions when aluminous materials are treated by defining the bath composition to the above range are as follows:

| Base solution | Metal salt    | Current type | Current density (A/dm <sup>2</sup> ) | Voltage (V) | Bath temperature (°C) | Time (min.) |
|---------------|---------------|--------------|--------------------------------------|-------------|-----------------------|-------------|
| Oxalic acid   | Ammonium salt | Direct       | 0.05-3                               | 5-160       | 10-40                 | 10-120      |
|               | Acetate       | do.          | 0.5-3                                | 5-130       | 10-40                 | 10-120      |
|               | Nitrate       | do.          | 0.5-5                                | 5-150       | 0-50                  | 10-120      |

oxidation, an alternating current must be applied and consequently there are problems in view of productivity and cost.

It is assumed that in the above described bath composition, oxalic acid contributes to the hue of the oxide coatings and that the metal salts provide an auxiliary

contribution. Furthermore, it is assumed that the metal salts mainly contribute to the luminosity range of the colored oxide coating.

The following examples are given for the purpose of illustration of this invention and are not intended as limitations thereof.

### Example 1

An aluminous material 1,100 was immersed in 7.5 percent by weight of an aqueous solution of sodium hydroxide at 80°C for 30 seconds and washed with water and then the thus treated aluminous material was immersed in 10 percent by weight of an aqueous solution of nitric acid to effect neutralization and washed with water.

The thus pretreated aluminous material was anodized as an anode in an electrolytic bath of an aqueous solution containing oxalic acid and stannous sulfate as shown in the following Table 1 at a temperature of 20±1°C, with a direct current of a current density of 2 A/dm<sup>2</sup> and a voltage of 30 – 105 V for 60 minutes to obtain colored oxide coatings showing greyish yellow as shown in Table 1.

Table 1

| Composition of electrolytic bath (% by weight) |                  | Voltage (V) | Thickness of coating (μ) | Color tone*    |
|------------------------------------------------|------------------|-------------|--------------------------|----------------|
| Oxalic acid                                    | Stannous sulfate |             |                          |                |
| 1                                              | 0.05             | 65-105      | 30                       | 7.5 GY 4.8/1.6 |
|                                                | 0.1              | 60-85       | 29                       | 2.6 G 4.6/1.9  |
|                                                | 0.1              | 55-75       | 31                       | 4.2 GY 5.4/1.7 |
| 3                                              | 0.3              | 45-65       | 29                       | 7.5 GY 4.7/1.6 |
|                                                | 0.5              | 40-55       | 28                       | 6.1 GY 4.2/1.6 |
| 5                                              | 0.75             | 35-45       | 30                       | 4.6 GY 5.5/1.5 |
|                                                | 1.0              | 35-40       | 30                       | 5.0 GY 4.9/1.6 |
| 10                                             | 1.5              | 30-35       | 31                       | 7.0 GY 6.2/1.4 |
|                                                | 2.0              | 30-33       | 30                       | 6.9 GY 6.2/1.4 |

\*Munsell notation

When ferrous sulfate was used instead of stannous sulfate, the similar results were obtained.

### Example 2

The same aluminous material as used in Example 1 was pretreated in the same manner as described in Example 1. The pretreated material was anodized as an anode in an electrolytic bath of an aqueous solution containing oxalic acid and titanium sulfate as shown in the following Table 2 at a temperature of 20±1°C with a direct current of a current density of 2 A/dm<sup>2</sup> and a voltage of 30 – 95 V for 60 minutes to obtain colored oxide coatings showing greyish yellow as shown in Table 2.

Table 2

| Composition of electrolytic bath (% by weight) |                  | Voltage (V) | Thickness of coating (μ) | Color tone*    |
|------------------------------------------------|------------------|-------------|--------------------------|----------------|
| Oxalic acid                                    | Titanium sulfate |             |                          |                |
| 1                                              | 0.05             | 60-95       | 28                       | 4.8 GY 4.7/1.7 |
|                                                | 0.1              | 55-75       | 29                       | 4.9 G 4.5/1.8  |
| 3                                              | 0.05             | 55-70       | 30                       | 5.5 GY 5.6/2.0 |
|                                                | 0.5              | 40-45       | 28                       | 7.3 GY 4.1/1.8 |
| 5                                              | 0.75             | 35-45       | 30                       | 7.8 GY 5.0/1.7 |

Table 2-Continued

| Composition of electrolytic bath (% by weight) |                  | Voltage (V) | Thickness of coating (μ) | Color tone*   |
|------------------------------------------------|------------------|-------------|--------------------------|---------------|
| Oxalic acid                                    | Titanium sulfate |             |                          |               |
| 7.5                                            | 0.75             | 35-40       | 27                       | 0.2 G 5.8/1.4 |
|                                                | 1.0              | 35-37       | 31                       | 0.2 G 5.6/1.4 |
| 10.0                                           | 1.0              | 30-35       | 30                       | 1.3 G 6.0/1.4 |
|                                                | 1.5              | 30-33       | 31                       | 1.5 G 6.0/1.2 |

\*Munsell notation

### Example 3

The same aluminous material as used in Example 1 was pretreated in the same manner as described in Example 1. The pretreated material was anodized as an anode in an electrolytic bath of an aqueous solution containing oxalic acid and manganese sulfate as shown in the following Table 3 at a temperature of 20±2°C with a direct current of a current density of 2 A/dm<sup>2</sup> and a voltage of 30 – 85 V for 60 minutes to obtain colored oxide coatings having a color tone ranging from amber to brown as shown in Table 3.

Table 3

| Composition of electrolytic bath (% by weight) |                   | Voltage (V) | Thickness of coating (μ) | Color tone*    |
|------------------------------------------------|-------------------|-------------|--------------------------|----------------|
| Oxalic acid                                    | Manganese sulfate |             |                          |                |
| 1                                              | 0.10              | 60-85       | 30                       | 2.5 G 4.4/1.6  |
| 1                                              | 0.20              | 55-75       | 31                       | 4 G 4.0/2.0    |
| 2                                              | 0.20              | 55-74       | 30                       | 9.3 GY 4.2/1.7 |
| 2                                              | 0.25              | 45-67       | 30                       | 9.0 GY 4.0/1.9 |
| 3                                              | 0.25              | 40-58       | 30                       | 8.0 GY 4.5/1.7 |
| 3                                              | 0.50              | 40-48       | 32                       | 7.5 GY 4.1/1.9 |
| 3.5                                            | 0.25              | 40-60       | 31                       | 5.0 GY 4.2/1.7 |
| 3.5                                            | 0.50              | 40-54       | 32                       | 6.8 GY 4.0/1.8 |
| 3.5                                            | 0.75              | 40-48       | 32                       | 7.2 GY 4.1/1.8 |
| 4.0                                            | 0.25              | 40-63       | 29                       | 2.9 GY 6.8/1.3 |
| 4.0                                            | 0.50              | 40-55       | 32                       | 5.2 GY 5.2/1.4 |
| 4.0                                            | 0.75              | 40-46       | 32                       | 6.8 GY 4.8/1.5 |
| 5.0                                            | 0.10              | 40-69       | 31                       | 2.0 GY 7.2/1.2 |
| 5.0                                            | 0.25              | 40-65       | 31                       | 3.8 GY 6.0/1.5 |
| 5.0                                            | 0.50              | 35-53       | 32                       | 4.2 GY 5.4/1.6 |
| 5.0                                            | 0.75              | 35-48       | 32                       | 4.5 GY 5.4/1.4 |
| 10.0                                           | 0.50              | 30-46       | 32                       | 3.0 GY 7.4/1.2 |
| 10.0                                           | 0.75              | 30-43       | 32                       | 4.2 GY 7.0/1.2 |
| 10.0                                           | 1.00              | 30-45       | 30                       | 6.6 GY 6.2/1.4 |

\*Munsell notation

### Example 4

In this example, the influence of the quality of aluminous material upon the color tone and thickness of the resulting coating was examined. Various aluminous materials as shown in the following Table 4 were anodized as an anode in an electrolytic bath of an aqueous solution containing 3 percent by weight of oxalic acid and 0.5 percent by weight of manganese sulfate at a temperature of 20±1°C with a direct current of a current density of 2 A/dm<sup>2</sup> for 60 minutes to obtain a result as shown in Table 4.

Table 4

| Alumi-<br>num<br>alloy<br>(AA) | Highest volt-<br>age at the<br>electrolysis<br>(V) | Thickness<br>of coating<br>( $\mu$ ) | Color tone* |         |
|--------------------------------|----------------------------------------------------|--------------------------------------|-------------|---------|
| 1100                           | 48                                                 | 32                                   | 7.4 GY      | 4.2/1.8 |
| 3003                           | 52                                                 | 30                                   | 3 G         | 4.2/1.9 |
| 5052                           | 49                                                 | 30                                   | 7.1 GY      | 4.6/1.6 |
| 6063                           | 49                                                 | 32                                   | 4.8 GY      | 5.8/1.4 |

\*Munsell notation

## Example 5

The same aluminous material as used in Example 1 was pretreated in the same manner as described in Example 1. The pretreated material was anodized as an anode in an electrolytic bath of an aqueous solution containing oxalic acid and ammonium phosphate as shown in the following Table 5 at a temperature of  $20 \pm 1^\circ\text{C}$  with a direct current of a current density of  $2 \text{ A/dm}^2$  and a voltage of  $60 - 150 \text{ V}$  for 60 minutes to obtain colored oxide coatings showing yellowish green as shown in Table 5.

Table 5

| Composition of<br>electrolytic bath<br>(% by weight) | Voltage<br>(V) | Thickness<br>of<br>coating<br>( $\mu$ ) | Color tone* |                |
|------------------------------------------------------|----------------|-----------------------------------------|-------------|----------------|
| Oxalic<br>acid                                       |                |                                         |             |                |
| 1                                                    | 0.05           | 80-150                                  | 28          | 5.9 GY 5.2/1.5 |
|                                                      | 0.1            | 85-140                                  | 30          | 7.7 GY 4.7/1.6 |
|                                                      | 0.1            | 60-85                                   | 30          | 2.7 GY 5.4/3.0 |
|                                                      | 0.3            | 70-85                                   | 31          | 1.3 GY 5.2/2.2 |
| 3                                                    | 0.5            | 75-90                                   | 31          | 0.3 GY 5.3/2.3 |
|                                                      | 0.75           | 85-95                                   | 32          | 2.5 GY 5.5/1.9 |
|                                                      | 1.0            | 95-110                                  | 31          | 7.4 GY 4.7/1.8 |
| 5                                                    | 1.5            | 80-90                                   | 29          | 2.8 GY 5.0/1.8 |
| 10                                                   | 1.5            | 60-70                                   | 29          | 7.4 Y 5.7/2.9  |

\*Munsell notation

## Example 6

The same aluminous material as used in Example 1 was pretreated in the same manner as described in Example 1. The pretreated material was anodized as an anode in an electrolytic bath of an aqueous solution containing oxalic acid and ammonium dichromate as shown in the following Table 6 at a temperature of  $20 \pm 1^\circ\text{C}$  with a direct current of a current density of  $2 \text{ A/dm}^2$  and a voltage of  $50 - 150 \text{ V}$  for 60 minutes to obtain colored oxide coatings having a color tone ranging from yellowish green to greyish yellow as shown in Table 6.

Table 6

| Composition of<br>electrolytic bath<br>(% by weight) | Voltage<br>(V) | Thickness<br>of<br>coating<br>( $\mu$ ) | Color tone* |                |
|------------------------------------------------------|----------------|-----------------------------------------|-------------|----------------|
| Oxalic<br>acid                                       |                |                                         |             |                |
| 1                                                    | 0.05           | 80-130                                  | 30          | 3.5 GY 5.7/1.6 |
|                                                      | 0.1            | 125-135                                 | 30          | 8.2 GY 5.6/1.1 |
|                                                      | 0.3            | 70-80                                   | 28          | 6.9 BG 5.6/1.6 |
|                                                      | 0.5            | 60-75                                   | 27          | 0.2 B 5.2/1.8  |
|                                                      | 0.05           | 50-80                                   | 29          | 8.6 Y 5.6/2.7  |

Table 6-Continued

| Composition of<br>electrolytic bath<br>(% by weight) | Voltage<br>(V) | Thickness<br>of<br>coating<br>( $\mu$ ) | Color tone* |                 |
|------------------------------------------------------|----------------|-----------------------------------------|-------------|-----------------|
| Oxalic<br>acid                                       |                |                                         |             |                 |
| 3                                                    | 0.3            | 50-80                                   | 29          | 0.1 GY 5.4/2.4  |
|                                                      | 0.7            | 50-135                                  | 30          | 2.9 GY 5.8/1.7  |
|                                                      | 1.5            | 100-150                                 | 31          | 1.0 GY 6.1/10.9 |
|                                                      | 0.05           | 45-60                                   | 28          | 7.0 Y 5.9/3.2   |
| 10                                                   | 0.3            | 45-60                                   | 28          | 7.4 Y 5.9/2.5   |
|                                                      | 0.7            | 50-60                                   | 28          | 7.1 Y 5.8/3.1   |
|                                                      | 1.5            | 50-85                                   | 29          | 9.1 Y 5.4/2.5   |
|                                                      | 3.0            | 80-135                                  | 31          | 4.6 GY 5.7/1.9  |

\* Munsell notation

## Example 7

The same aluminous material as used in Example 1 was pretreated in the same manner as described in Example 1. The pretreated material was anodized as an anode in an electrolytic bath of an aqueous solution containing oxalic acid and manganese acetate as shown in the following Table 7 at a temperature of  $20 \pm 1^\circ\text{C}$  with a direct current of a current density of  $2 \text{ A/dm}^2$  and a voltage of  $45 - 130 \text{ V}$  for 60 minutes to obtain colored oxide coatings having a color tone ranging from yellow to dark yellowish green as shown in Table 7.

Table 7

| Composition of<br>electrolytic bath<br>(% by weight) | Voltage<br>(V) | Thickness<br>of<br>coating<br>( $\mu$ ) | Color tone*    |                |
|------------------------------------------------------|----------------|-----------------------------------------|----------------|----------------|
| Oxalic<br>acid                                       |                |                                         |                |                |
| 1                                                    | 0.05           | 80-120                                  | 29             | 5.7 Y 5.5/1.7  |
|                                                      | 0.1            | 80-115                                  | 30             | 2.4 GY 5.7/1.8 |
|                                                      | 0.3            | 85-130                                  | 30             | 4.4 GY 5.5/1.9 |
|                                                      | 0.05           | 60-75                                   | 29             | 7.3 Y 5.8/2.7  |
| 3                                                    | 0.1            | 60-80                                   | 29             | 7.7 Y 5.7/2.7  |
|                                                      | 0.3            | 100-130                                 | 31             | 8.8 Y 5.7/2.7  |
|                                                      | 0.5            | 110-130                                 | 31             | 5.1 GY 5.5/1.6 |
|                                                      | 0.7            | 130<br>(constant)                       | 32             | 5.4 GY 5.4/1.2 |
| 50                                                   | 1.0<br>do.     | 32                                      | 5.2 GY 5.6/0.6 |                |
|                                                      | 0.05           | 50-60                                   | 28             | 7.2 Y 5.7/3.1  |
| 5                                                    | 0.7            | 50-65                                   | 28             | 8.2 Y 5.6/2.9  |
| 10                                                   | 0.05           | 45-55                                   | 27             | 7.1 Y 5.9/3.1  |
|                                                      | 0.7            | 50-60                                   | 28             | 3.6 Y 5.6/3.2  |

\* Munsell notation

## Example 8

The same aluminous material as used in Example 1 was pretreated in the same manner as described in Example 1. The pretreated material was anodized as an anode in an electrolytic bath of an aqueous solution containing oxalic acid and chromium acetate as shown in the following Table 8 under the same condition and procedure as described in Example 1 to obtain colored oxide coatings having a color tone ranging from yellow to dark yellowish green as shown in Table 8.

Table 8

| Composition of electrolytic bath (% by weight) |                  | Voltage (V) | Thickness of coating ( $\mu$ ) | Color tone*    |
|------------------------------------------------|------------------|-------------|--------------------------------|----------------|
| Oxalic acid                                    | Chromium acetate |             |                                |                |
| 1                                              | 0.05             | 75-130      | 31                             | 4.3 GY 5.6/1.8 |
|                                                | 0.05             | 60-80       | 30                             | 8.8 Y 5.6/2.6  |
|                                                | 0.1              | 60-80       | 30                             | 9.0 Y 5.6/2.6  |
| 3                                              | 0.3              | 60-80       | 30                             | 8.5 Y 5.6/2.7  |
|                                                | 0.5              | 65-110      | 31                             | 1.0 GY 5.2/2.4 |
|                                                | 1.0              | 65-105      | 31                             | 10 Y 5.4/2.5   |
| 5                                              | 0.05             | 55-70       | 28                             | 5.1 GY 5.6/2.7 |
| 7.5                                            | 0.05             | 50-60       | 28                             | 5.6 Y 5.9/3.1  |
| 10.0                                           | 0.05             | 45-55       | 27                             | 7.2 Y 5.8/3.1  |

\* Munsell notation

## Example 9

The same aluminous material as used in Example 1 was pretreated in the same manner as described in Example 1. The pretreated material was anodized as an anode in an electrolytic bath of an aqueous solution containing oxalic acid and ferric nitrate as shown in the following Table 9 at a temperature of  $20 \pm 1^\circ\text{C}$  with a direct current of a current density of  $2 \text{ A/dm}^2$  and a voltage of  $45 - 110 \text{ V}$  for 60 minutes to obtain colored oxide coatings showing greyish yellow as shown in Table 9.

Table 9

| Composition of electrolytic bath (% by weight) |                | Voltage (V) | Thickness of coating ( $\mu$ ) | Color tone*    |
|------------------------------------------------|----------------|-------------|--------------------------------|----------------|
| Oxalic acid                                    | Ferric nitrate |             |                                |                |
| 1                                              | 0.05           | 70-110      | 28                             | 6.4 GY 5.7/1.7 |
| 3                                              | 0.05           | 55-75       | 30                             | 1.0 GY 5.7/2.4 |
|                                                | 0.1            | 60-80       | 29                             | 2.6 GY 5.5/2.1 |
| 5                                              | 0.3            | 55-65       | 30                             | 3.4 GY 5.6/1.8 |
|                                                | 0.5            | 65-65       | 30                             | 3.4 GY 5.6/1.8 |
|                                                | 0.5            | 65-75       | 31                             | 0.2 G 4.9/1.5  |
| 7.5                                            | 0.5            | 45-55       | 31                             | 2.5 GY 5.9/1.9 |
| 10.0                                           | 0.75           | 45-50       | 29                             | 2.5 GY 5.8/1.9 |

\* Munsell notation

## Example 10

The same aluminous material as used in Example 1 was pretreated in the same manner as described in Example 1. The pretreated material was anodized as an anode in an electrolytic bath of an aqueous solution containing oxalic acid and chromium nitrate as shown in the following Table 10 at a temperature of  $22 \pm 1^\circ\text{C}$  with a direct current of a current density of  $2 \text{ A/dm}^2$  and a voltage of  $45 - 110 \text{ V}$  for 60 minutes to obtain colored oxide coatings showing greyish and yellowish green as shown in Table 10.

## 8

Table 10

| Composition of electrolytic bath (% by weight) |                  | Voltage (V) | Thickness of coating ( $\mu$ ) | Color tone*    |
|------------------------------------------------|------------------|-------------|--------------------------------|----------------|
| Oxalic acid                                    | Chromium nitrate |             |                                |                |
| 1                                              | 0.05             | 70-110      | 29                             | 6.7 GY 5.7/1.8 |
| 3                                              | 0.05             | 60-75       | 29                             | 1.9 GY 5.6/2.1 |
|                                                | 0.10             | 60-80       | 30                             | 5.0 GY 5.6/2.6 |
| 5                                              | 0.30             | 50-60       | 28                             | 2.0 GY 5.9/2.3 |
| 10                                             | 0.50             | 45-50       | 28                             | 1.2 GY 6.2/2.1 |
|                                                | 0.75             | 45-50       | 29                             | 1.0 GY 6.2/2.1 |

\* Munsell notation

As described above, in the method of the present invention, an aluminous material which has been previously degreased and washed with water is anodized in an electrolytic aqueous bath containing oxalic acid and a metal salt to obtain a colored oxide coating. Therefore, the method of the present invention has the following merits.

1. Electrolyte is inexpensive.
2. High technique is not required.
3. Efficiency is high.
4. Oxide coatings having a broad range of color tone from yellow to brown can be obtained.

That is, the above merit (1) is that the electrolytic bath is composed of usual chemicals and therefore the cost is inexpensive, and the above merit (2) is that satisfactorily colored oxide coatings can be easily obtained by using an electrolytic bath maintained at room temperature, and therefore the bath can be easily controlled. Accordingly, in the method of the present invention, aluminous materials can be treated in the same manner as in the case of conventional anodic oxidation process. Moreover, the oxidized coating obtained by the method of the present invention is excellent in the corrosion resistance, abrasion resistance and weather resistance.

What is claimed is:

1. A method of producing colored oxide coatings ranging from yellow to brown on aluminum or aluminum alloy, which consists essentially of electrolytically anodizing with direct current, an aluminum material selected from the group consisting of aluminum and an alloy thereof in an aqueous solution of 0.5 - 10.0 percent by weight of oxalic acid and 0.05 - 4.0 percent by weight of a salt selected from the group consisting of ammonium phosphate, ammonium dichromate, a metal acetate and a metal nitrate at a temperature of between  $0^\circ$  and  $50^\circ\text{C}$ ; a voltage of between 5-160 volts, a current density of between  $0.05 - 5 \text{ A/dm}^2$ , and for a time of between 10-120 minutes.
2. A method as claimed in claim 1, wherein said acetate is selected from the group consisting of manganese acetate and chromium acetate.
3. A method as claimed in claim 1, wherein said metal nitrate is selected from the group consisting of ferric nitrate and chromium nitrate.
4. A method of producing colored oxide coatings ranging from yellow to brown on aluminum or aluminum alloy, which consists essentially of electrolytically anodizing with direct current, an aluminum material selected from the group consisting of aluminum and an alloy thereof in an aqueous solution of 0.5 - 10.0 percent by weight of oxalic acid and 0.05 - 4.0 percent by weight of a salt selected from the group consisting of ammonium phosphate, ammonium dichromate, a metal acetate and a metal nitrate at a temperature of between  $0^\circ$  and  $50^\circ\text{C}$ ; a voltage of between 5-160 volts, a current density of between  $0.05 - 5 \text{ A/dm}^2$ , and for a time of between 10-120 minutes.

weight of a salt selected from the group consisting of ammonium phosphate, ammonium dichromate, manganese acetate, chromium acetate, ferric nitrate and chromium nitrate at a temperature of between 0° and 50°C; a voltage of between 5-160 volts, a current density of between 0.05 - 5 A/dm<sup>2</sup>, and for a time of between 10-120 minutes.

5. A method as claimed in claim 4, wherein the

amount of said ammonium salt is 0.05 - 4.0 percent by weight.

6. A method as claimed in claim 1, wherein the amount of said acetate is 0.05 - 1.5 percent by weight.

5 7. A method as claimed in claim 4, wherein the amount of said metal nitrate is 0.05 - 0.7 percent by weight.

\* \* \* \* \*

10

15

20

25

30

35

40

45

50

55

60

65